

1

3,383,312

## STABLE, FLUID, SOAP THICKENED OIL LUBRICANT COMPOSITIONS

Walter J. Coppock, Wallingford, Pa., assignor to Sun Oil Company, Philadelphia, Pa., a corporation of New Jersey  
No Drawing. Filed Dec. 21, 1964, Ser. No. 420,092  
8 Claims. (Cl. 252—36)

In one aspect this invention is a method of preparing fluid, soap thickened oil lubricants which are stable in that there is no tendency of the soap to separate from the oil during storage or use. Stability is achieved by incorporating a small amount of a cyclic aluminum oxide trimer into the lubricant. In another aspect the invention is stable, fluid, soap thickened oil lubricants comprising lubricating oil, soap, and the aforesaid trimer.

Fluid lubricant compositions comprising a major amount of lubricating oil and 0.1—2.5% soap dispersed therein are known. The compositions are fluid, i.e., pourable, as opposed to being grease, i.e., semi-solid, compositions. The purpose of the soap is to increase the apparent viscosity of the oil and the composition is used, for example, in lubricating exposed gear teeth or exposed bearings, i.e., surfaces where in the absence of the soap the oil would tend to drip off or otherwise escape from the surface to be lubricated. A number of other applications of soap thickened oil fluid lubricants are also known; see, e.g., U.S. Patent 3,071,547.

In most soap thickened oil fluid lubricants the oil is a mineral lubricating oil and the soap is a metal salt of a fatty acid. Although such lubricants have a number of desirable properties they have an undesirable characteristic in that the soap tends to settle out of the oil. For example, if a drum of a homogeneous fluid lithium stearate thickened oil is stored for six months and the contents then examined, it will often be found that the material at the bottom of the drum is mainly oil and the material at the top of the drum is mainly soap. This storage instability is an obvious disadvantage and a means of preventing same is desired.

It has now been found that fluid lubricants comprising mineral lubricating oils thickened with metal soaps of fatty acids can be stabilized against separation of the soap by the incorporation therein of a small amount of a cyclic aluminum oxide trimer having certain characteristics more fully defined hereinafter. In one aspect the invention is fluid, stable, oil-soap-trimer compositions. In another aspect it is a method of preparing same.

It is recognized that in fluid, soap thickened oil lubricants, as in greases, the soap is not dissolved, at least at room temperature, in the oil (except for possibly an insignificant amount) but rather is dispersed therein. Consequently when it is stated herein that the soap separates from the oil it is obviously not meant that the soap comes out of the solution. What is meant is that the dispersed soap settles so that what was initially a homogeneous dispersion becomes non-homogeneous or, in extreme cases, two distinct layers, a soap layer and an oil layer.

The oil component of the compositions of the invention is a mineral lubricating oil. Being a mineral oil it will also be a hydrocarbon oil. Any particular type of mineral oil is suitable so long as it has lubricating properties. Thus the oil can be paraffinic, naphthenic, etc. It can be a straight distillate oil, a solvent refined oil, etc. The viscosity of the oil will vary depending upon the intended application but will usually be 80—3500 S.U.S. at 100° F., more frequently 100—3000 S.U.S. at 100° F. The VI of the oil will depend upon the type of oil and its method of preparation but will usually be 0—100. The amount of oil in the compositions of the invention will be 95—99.8% based on the total composition, i.e., on the oil, soap, and

2

trimer. All percentages and parts herein are by weight.

The soap component of the compositions of the invention is a fatty acid metal soap. The fatty acid should contain 12—22 carbon atoms and is preferably an unsubstituted fatty acid such as stearic, palmitic, etc. but it can also be a substituted fatty acid such as 12-hydroxy stearic acid. The preferred fatty acid is stearic acid. The metal component of the soap can be any of the conventional soap forming metals such as sodium, lithium, barium, calcium, aluminum, etc. The tendency of the soap to separate from a fluid mineral oil lubricant is not dependent upon the specific metal present in the soap. For economic reasons the alkali and alkaline earth metals are preferred for the present purpose. Of these the alkali metals are preferred, especially lithium since oils thickened with lithium soaps have good resistance to water and high temperatures.

The amount of soap used in the compositions will depend upon the intended application thereof but will usually be 0.1—2.5% based on the total composition. In any event the amount of soap will be sufficient to increase the apparent viscosity of the oil. The viscosity is referred to as apparent because although addition of the soap to the oil increases the viscosity of the oil as determined by conventional analytical methods, when the soap thickened oil is subjected to shear its viscosity reduces to that of the oil alone. In other words, the soap thickened oil is non-Newtonian fluid. The amount of soap will normally be such that the final fluid oil-soap-trimer composition has a MacMichael viscosity at 70° F. (oil cup) of 2—25, the MacMichael viscosity being used instead of S.U.S. viscosity because S.U.S. viscosities on dispersions are not reliable. The maximum amount of soap is limited to 2.5% because above this amount the soap thickened oil is usually of grease consistency rather than being fluid. The present invention does not include grease compositions because with these there is no soap separation problem. In other words, in an oil thickened to grease consistency with a fatty acid metal soap there is no problem of the soap settling out. This problem does exist, however, in a fluid soap thickened oil. The preferred amount of soap for the present purpose is 0.5—1.5%.

The substituted cyclic aluminum oxide trimer which is included in the compositions of the invention in order to prevent separation of the soap from the oil has the structure



wherein R in at least one instance is an acylate anion ( $\text{RCOO}^-$ ) of an aliphatic monocarboxylic acid containing 12—22 carbon atoms and in any remaining instances is an alkoxy anion ( $\text{RO}^-$ ) of an alcohol containing 1—10 carbon atoms such as ethanol, hexanol, octanol, isopropanol, heptanol, sec-butanol, etc. Preferably the alcohol from which the alkoxy anion is derived contains 2—5 carbon atoms and more preferably is isopropanol. Examples of suitable acids from which the acylate anion is derived are stearic acid, palmitic acid, 12-hydroxy stearic, etc. It is not necessary that the acid from which the acylate anions in the trimer are derived be the same as the acid used to form the soap which is present in the compositions of the invention. Furthermore, it is not necessary that all acylate anions in the trimer be the same or that all alkoxy anions in the trimer be the same. Although it is sufficient if only one R in (I) above is an acylate anion of the type described preferably at least 2 R's, more preferably all R's, are acylate anions.

The substituted cyclic aluminum oxide trimer and the method of making same are described in detail in U.S. Patent No. 2,979,497, issued to Jacobus Rinse. As described in this patent, an aliphatic monocarboxylic acid, an aluminum alkoxide, and water are mixed and then held at a temperature of 176°-248° F. until formation and liberation of alcohol ceases, after which the temperature is raised to and maintained at about 356° F. until further formation and liberation of alcohol ceases. The product is the substituted cyclic aluminum oxide trimer. The substitutions will be either acylate or alkoxy anions depending upon the mole ratios of the reactants used. For example, if the mole ratio of acid to aluminum alkoxide to water is 1:1:1, the product will be a triacylate cyclic aluminum oxide trimer,



If the mole ratio of acid to aluminum alkoxide to water is 2:3:3, the product will be a diacylate alkoxy cyclic aluminum oxide trimer,



Further variations in mole ratios of the ingredients result in further variations of the substitutions on the cyclic aluminum oxide trimer.

The amount of the substituted cyclic aluminum oxide trimer, herein referred to as the trimer, should be in the range of 0.1-2.5% based on the total composition since amounts within this range are effective to prevent separation of the soap from the oil. Preferably the amount used is 0.5-1.5%. As a general rule the amount of trimer required to prevent separation of the soap decreases as the amount of soap decreases.

The trimer must be incorporated into the compositions of the invention in a certain manner if the stabilizing effect of the trimer is to be realized. The trimer can be satisfactorily incorporated at any time during the preparation of the soap thickened oil or at any time thereafter so long as the composition is heated to at least 200° F., preferably at least 300° F., after the addition of the trimer thereto. Thus if the trimer is merely added to and mixed with a fluid, soap thickened oil at room temperature the soap in the resulting three component composition will still settle out during storage. If, however, the resulting three component composition is heated to at least 200° F. and then cooled to room temperature separation of the soap thereafter will not occur. The reason why the composition containing the trimer must reach a temperature of at least 200° F. to be stable is not known but such has nevertheless been found to be the case. It is apparently not necessary that the composition be held at a temperature of at least 200° F. for any certain prescribed period because it has been found that merely heating to, say, 210° F. and then immediately cooling to room temperature is sufficient. In any event, in a commercial operation the composition would usually be above 200° F. for 5-10 minutes because of the characteristics of the equipment utilized and this is the preferred procedure.

In actual practice it will usually be much more convenient to incorporate the trimer during the preparation of the soap thickened oil composition. Soap thickened oils are conventionally prepared by mixing the soap with a minor proportion, usually 1/4-1/2, of the total oil at about room temperature. Only a minor amount of the oil is used in order to minimize the oil decoloration which occurs because of the subsequent heating. The soap-oil

5 mixture is then heated with agitation to effect dissolution of the soap in the oil and the mixture is then cooled with agitation while adding the remainder of the oil thereto. During the cooling the solubility of the soap in the oil decreases and most of the soap comes out of the oil. Normally all the remaining oil is added before a temperature of 180° F. in the cooling step is reached. If any additives such as oxidation inhibitors are to be included in the composition they are normally added at about 180°-200° F. After all ingredients are present cooling continues until a temperature below 100° F., usually room temperature, is reached.

10 The soap-oil mixture is normally agitated during the entire cooling cycle, i.e., even after all the oil is in and a uniform soap-oil mixture achieved. This is done in order to prevent any gelation which might otherwise occur. Agitation beyond that required to make a homogeneous soap-oil mixture is not essential, however, for even if any gelation occurs the gel can be broken up and a fluid 15 lubricant obtained by merely agitating the soap-oil mixture.

20 The soap component can be preformed or can be formed in situ in the oil. For example, stearic acid and lime can be mixed with a minor proportion of the oil. During the subsequent heating the lime and acid react to form calcium stearate and water, the latter being evaporated during the heating step.

25 The temperature to which the soap-oil mixture must be heated to dissolve the soap in the oil in a reasonable length of time will vary depending mainly upon the metal component of the soap. For alkaline earth metals a temperature of 250°-350° F. is usually sufficient. With lithium soaps a temperature of 350°-425° F. is preferred but with other alkali metal soaps lower temperatures of 300°-400° 30 F. are satisfactory. In any event dissolution of the soap in the oil can be readily determined visually.

35 One convenient method of incorporating the trimer is to add the trimer to the oil at the same time the soap is added. The trimers suitable for the present purpose are oily liquids completely miscible with mineral lubricating oils. Since the resulting mixture will always be heated to above 200° F. to dissolve the soap in the oil this heating will simultaneously realize the stabilizing effect of the trimer. Alternatively, the trimer can be added at any time during the heating or cooling operations so long as a temperature of at least 200° F., preferably at least 300° F., is reached after addition of the trimer.

40 One precaution should be observed in adding the trimer when the soap is formed in situ in the oil because of the fact that this in situ technique results in the formation of water. At high, e.g., 10-15% concentrations of trimer in oil the presence of water sometimes tends to convert the oil to grease. Furthermore this grease usually cannot be converted to a fluid lubricant by merely agitating the grease because of the relatively large amount of soap present. Thus this situation is not the same as the case mentioned previously in which gelation of the oil occurs during the cooling cycle due to lack of agitation. Since only a minor proportion of the oil, usually 1/4-1/2, is normally present initially, the concentration of trimer will be substantially higher initially than in the final composition. In order to avoid converting the oil to a grease the trimer should not be added to the oil until any water present is removed. This presents no serious obstacle because the oil will of course be dehydrated during the heating step. If the soap is preformed this problem of course does not arise.

45 The following examples illustrate the invention more specifically.

#### EXAMPLE 1

50 35.0 parts of a paraffinic solvent refined distillate oil having a viscosity of 100 S.U.S. at 100° F. and a VI of 90 is charged to a jacketed vessel equipped with a paddle type agitator. Steam or cold water can be supplied to the jacket for heating or cooling of the contents of the vessel.

With the agitator running and the oil at 75° F. 0.7 part lithium stearate is added to the oil and the resulting mixture is heated over a period of 2 hours to 400° F. at which temperature the lithium stearate is dissolved in the oil. When the temperature reaches 400° F. the steam is shut off and the cooling water turned on. Just after cooling begins 63.9 additional parts of oil is charged to the vessel and the contents of the tank are cooled to 75° F. over a period of 2 hours. At 180° F. in the cooling step 0.4 part of dibutyl-para-cresol, an oxidation inhibitor, is charged to the vessel. The agitator is running during the entire cooling step.

A conventional 55 gallon drum containing sample taps at the bottom, 17 inches up from the bottom (hereinafter the middle), and 34 inches up from the bottom (hereinafter the top), is filled to a depth of 35 inches with the oil prepared as described above. Immediately after filling a small sample is withdrawn from each of the sample taps and the viscosity of each sample is determined. Each sample has a MacMichael viscosity at 70° F. of 13. The drum is then closed and is placed in storage at 75° F. After 2 months' storage another sample is withdrawn from each tap and the viscosity of each sample is determined. The results are as follows.

| Location: | MacMichael viscosity at 70° F. |
|-----------|--------------------------------|
| Top       | 30                             |
| Middle    | 20                             |
| Bottom    | 2                              |

It is evident from this data that the soap thickened oil has poor storage stability.

#### EXAMPLE 2

A soap thickened oil is prepared by the procedure of Example 1 except that instead of using 35 parts oil 34.5 parts are used and 0.5 part cyclic aluminum oxide trimer is added to the oil simultaneously with the lithium stearate soap. The trimer has the structure of (I) supra wherein 2 R's are stearate and 1 R is isopropoxy. In other words the trimer is a distearate isopropoxy cyclic aluminum oxide trimer.

The soap thickened oil prepared in this manner is charged to a 55 gallon drum similar to that used in Example 1 and tested in the same manner as in Example 1. The results are as follows: Immediately after filling the drum each sample has a MacMichael viscosity at 70° F. of 13. After 2 months' storage the three samples have viscosities as follows.

| Location: | MacMichael viscosity at 77° F. |
|-----------|--------------------------------|
| Top       | 13                             |
| Middle    | 13                             |
| Bottom    | 13                             |

It is evident from the above results that the inclusion of the trimer in the composition has resulted in a storage stable soap thickened oil. When other soaps, oil, and trimers as described herein are used the results are substantially the same.

The invention claimed is:

1. A stable, fluid, soap thickened oil lubricant composition comprising a major amount of mineral lubricating oil, 0.1-2.5%, sufficient to increase the apparent viscosity of said oil, of a fatty acid metal soap dispersed in said oil, and 0.1-2.5%, sufficient to reduce the tendency of said soap to separate from said oil, of a substituted cyclic aluminum oxide trimer having the structure



wherein R in at least one instance is an acylate anion of an aliphatic monocarboxylic acid containing 12-22 carbon atoms and in any remaining instances is an alkoxy anion of an alcohol containing 1-10 carbon atoms, the amount and percentages being by weight of the total composition.

2. The composition according to claim 1 wherein all R's are acylate anions.

3. The composition according to claim 1 wherein the amount of said soap is 0.5-1.5% and the amount of said trimer is 0.5-1.5%.

4. The composition according to claim 1 wherein said metal is lithium.

5. A method of preparing a fluid, soap thickened mineral oil lubricant composition which is stable in that the tendency of the soap to separate from the oil is reduced which comprises forming a mixture of a minor proportion of the oil in said composition, a fatty acid metal soap in the amount of 0.1-2.5% based on said composition, said amount being sufficient to increase the apparent viscosity of the oil in said composition, heating said mixture to dissolve the soap in oil, cooling said mixture to below 100° F. while adding additional oil thereto during at least a portion of said cooling, and adding to said mixture a stabilizing amount, in the range of 0.1-2.5%, based on said composition, of a cyclic aluminum oxide trimer having the structure



wherein R in at least one instance is an acylate anion of an aliphatic monocarboxylic acid containing 12-22 carbon atoms and in any remaining instances is an alkoxy anion of an alcohol containing 1-10 carbon atoms, said adding being at a time in the forming-heating-cooling operation such that the resulting oil-soap-trimer mixture reaches a temperature of at least 200° F.

6. The method according to claim 5 wherein all R's are acylate anions.

7. The method according to claim 5 wherein said metal is lithium.

8. The method according to claim 5 wherein said oil-soap-trimer mixture reaches a temperature of at least 300° F.

#### References Cited

##### UNITED STATES PATENTS

|           |         |               |       |          |
|-----------|---------|---------------|-------|----------|
| 2,489,300 | 11/1949 | Leyda         | ----- | 252-36   |
| 2,744,074 | 5/1956  | Theobald      | ----- | 260-2    |
| 2,859,181 | 11/1958 | Jordan et al. | ----- | 252-36   |
| 2,883,341 | 4/1959  | Allison       | ----- | 252-36   |
| 2,913,409 | 11/1959 | Remes et al.  | ----- | 252-28   |
| 2,979,497 | 4/1961  | Rinse         | ----- | 260-97.5 |
| 3,055,828 | 9/1962  | Wiley         | ----- | 252-35   |
| 3,216,935 | 11/1965 | Morway et al. | ----- | 252-39   |
| 3,231,495 | 1/1966  | Morway et al. | ----- | 252-39   |

DANIEL E. WYMAN, Primary Examiner.

I. VAUGHN, Assistant Examiner.